

## UNITED STATES PATENT OFFICE

2,672,411

## GELATIN BLASTING EXPLOSIVES

James Taylor, Ardrossan, and James V. Gregg,  
West Kilbride, Scotland, assignors to Imperial  
Chemical Industries Limited, a corporation of  
Great Britain

No Drawing. Application May 31, 1950,  
Serial No. 165,368

Claims priority, application Great Britain  
July 29, 1949

4 Claims. (Cl. 52—13)

1

The present invention relates to improvements in gelatine blasting explosive compositions of the kind comprising a vegetable tissue material and an oxidising agent distributed through a continuous matrix of a liquid explosive nitric ester-nitrocellulose jelly.

It is known that gelatine blasting explosive compositions comprising woodmeal and oxidising salts such as sodium nitrate distributed through a liquid explosive nitric ester-nitrocellulose jelly fail to propagate their detonation satisfactorily when initiated by commercial detonators in shot-holes where they are subjected to hydrostatic pressures substantially in excess of 3 atmospheres. It is also known that the replacement or partial replacement of woodmeal in such explosive compositions by porous vegetable tissue materials of unusually low bulk density, for example, bagasse, flaked steam treated cereal grain products, and ground-cork, increases the sensitivity and velocity of detonation at atmospheric pressure of the resulting gelatine blasting explosive compositions and enables them to be detonated at somewhat higher hydrostatic pressures, but the incapacity for and velocity of detonation still diminish markedly as the hydrostatic pressure is increased, with the result that these explosives cannot be relied upon to detonate satisfactorily in bore-holes sunk under depths of oil or water as great as would frequently be encountered in well blasting or seismic prospecting operations. The aeration resulting from the mechanical mixing operation in the production of liquid explosive nitric ester-nitrocellulose gelatine blasting explosives persisting for some time after the mixing operation is known to have the effect of rendering the sensitivity to detonation of the freshly made gelatine blasting explosive compositions higher than that possessed by it after the density of the composition has risen to its normal value as a result of the escape of air bubbles. The favourable effect on sensitivity to detonation and velocity of detonation experienced as a result of the employment of porous vegetable tissue ingredients of unusually low bulk density is usually attributed to the entrapment of air in their pores or to their levitating effect on the composition, and the deterioration in these properties of the gelatine explosives containing them under increasing hydrostatic pressure may likewise be attributed to the reduction in volume of the entrapped air as a result of the pressure transmitted through the continuous liquid nitric ester-nitrocellulose jelly to the structure of the vegetable tissue

2

material, whether or not this results in its actual collapse. It will be readily understood that the flimsier the structure of the porous vegetable tissue material the more easily will the beneficial effects experienced at atmospheric pressure as a result of its use in a liquid nitric ester-nitrocellulose gelatine blasting explosive composition be lost when the explosive is subjected to hydrostatic pressure. Moreover there is a limit to the amount of porous vegetable tissue material of unusually low density that can be incorporated into a gelatine blasting explosive without destroying the continuity of the matrix essential for the waterproof properties and bulk strength characteristic of gelatine explosives.

It is an object of the present invention to provide gelatine blasting explosive compositions of the kind comprising a porous vegetable tissue material and an oxidising salt distributed through a continuous matrix of a liquid explosive nitric ester-nitrocellulose jelly which will detonate satisfactorily under greater hydrostatic pressures than can be attained by the use of the customary porous vegetable tissue materials of unusually low bulk density.

According to the present invention a gelatine blasting explosive of the kind comprising a porous vegetable material ingredient and an oxidising salt distributed through a continuous matrix of a liquid explosive nitric ester-nitrocellulose jelly is characterised in that the porous vegetable material consists of dried substantially deproteinised, de-oiled peanut meal obtained by aqueous alkaline extraction washing and de-watering of a peanut product from which the oil has been removed in known manner as for instance by expression or by extraction with a volatile solvent or by expression followed by extraction with a volatile solvent. The dried substantially de-proteinised de-oiled peanut meal, which is preferably one made from peanuts from which the brown testa has first been removed, is a porous material consisting mainly of cellulose, and constitutes a commercially available by-product from the manufacture of peanut protein. Peanut protein is used in the manufacture of certain protein textile artificial filaments. The deproteinised de-oiled peanut meal is desirably screened so as to reject any meal passing a 100 B. S. S. screen or retained on a 16 B. S. S. screen. Advantageously the washed and centrifuged material may be worked through a coarse screen before the final drying step and if necessary may be milled thereafter before the final screening.

The de-proteinised de-oiled peanut meal so obtained has a bulk density of approximately 0.46 gram per cc. under a packing pressure of 25 lbs. per sq. in. and approximately 0.51 gram per cc. under a packing pressure of 75 lbs. per sq. in. and its density is thus higher than that of ordinary woodmeal, which exhibits bulk densities of approximately 0.35 and approximately 0.41 under these pressures. Its absorbency for nitroglycerine under a pressure of 75 lbs. per sq. in. is approximately 150%, the corresponding figure for ordinary woodmeal being about 250%. The corresponding approximate figures for bulk density and nitroglycerine absorption for bagasse and for ground cork are respectively as follows:

Density at 25 lbs. pressure—0.17 and 0.16 gm. per cc.

Density at 75 lbs. pressure—0.25 and 0.29 gm. per cc.

Absorbency—328% and 110%.

It contains 44% carbon, 4.5% nitrogen and 6% hydrogen.

In putting the invention into effect the de-proteinised de-oiled peanut meal may be incorporated into the explosive composition in the conventional manner employed for other vegetable tissue materials. The oxidising salt may be an alkali metal nitrate but it is also possible to employ the de-proteinised de-oiled peanut meal in ammonium nitrate gelatine explosives.

The invention will be further understood by reference to the example, in which the percentages are by weight. In this example reference is made to a test in which three cartridges in file each 10.5 in. long and of 2 in. diameter separated by gaps  $\frac{1}{2}$  in. in length and enclosed in a telescopic cardboard tube are fired under varying water pressures and the velocity of detonation of the third cartridge is observed. In these tests the cardboard container is punctured so as to ensure that the cartridges, which are enclosed in conventional waxed paper wrappers, are separated from one another by water, and the first cartridge in each test is provided with a No. 8 commercial lead azide aluminum detonator. The cartridges are immersed for  $\frac{1}{2}$  an hour before they are fired. The results of similar tests on cartridges of gelatine compositions of similar plasticity containing other vegetable tissue materials are also given, and it will be seen that the cartridges of the explosive in accordance with the present invention exhibit a superior constancy of velocity of detonation under pressures ranging from 50 lbs. per sq. in. upwards and can be detonated satisfactorily under higher pressures.

#### Example

The ingredients of the gelatine explosive composition are as follows:

|                                                                                         | Per cent |
|-----------------------------------------------------------------------------------------|----------|
| Mixture of nitroglycerine and ethylene glycol dinitrate in the ratio 80:20 by weight    | 57.5     |
| "Blasting Soluble" nitrocellulose                                                       | 2.5      |
| De-proteinised de-oiled peanut meal passing 16 and retained by 100 mesh B. S. S. screen | 13.0     |
| Sodium nitrate                                                                          | 26.4     |
| Chalk                                                                                   | 0.3      |
| Di-ammonium hydrogen phosphate                                                          | 0.3      |

The ingredients are mixed in known manner

in a McRobert mixer until the nitrocellulose has become well gelatinised and the other ingredients are well distributed through the jelly. The density of the composition after storage for two days is 1.51 grams per cc. In the triple cartridge test under varying heads of water the explosive composition gives the following figures for the velocity of detonation in the third cartridge:

|                      | Meters per sec. |
|----------------------|-----------------|
| 50 lbs. per sq. in.  | 2400            |
| 100 lbs. per sq. in. | 2210            |
| 200 lbs. per sq. in. | 2580            |
| 250 lbs. per sq. in. | 2580            |
| 300 lbs. per sq. in. | 2580            |
| 450 lbs. per sq. in. | 2500            |

The explosive is thus suitable for use in seismic prospecting and for well blasting at substantial depths, using a No. 8 commercial lead azide tetryl aluminum detonator.

By way of comparison the compositions, densities, and performances in the triple cartridge tests are given below for two gelatine explosive compositions not in accordance with the invention containing the same percentages of liquid explosive nitric ester and nitrocellulose of the same consistency. These compositions are made by using vegetable tissue materials of unusually low density, and by adjusting the proportion of sodium nitrate to compensate for the different absorptive capacities of the vegetable tissue materials employed.

|                                                               | Percent | Percent |
|---------------------------------------------------------------|---------|---------|
| 80:20 mixture of nitroglycerine and ethylene glycol dinitrate | 57.5    | 57.5    |
| "Blasting Soluble" nitrocellulose                             | 2.5     | 2.5     |
| Bagasse                                                       | 8.0     |         |
| Starch                                                        |         | 6.0     |
| Flaked steam treated cereal grained product                   |         | 6.0     |
| Sodium nitrate                                                | 31.4    | 29.4    |
| Chalk                                                         | 0.3     | 0.3     |
| Di-ammonium hydrogen phosphate                                | 0.3     | 0.3     |
| Density in gm./cc.                                            | 1.43    | 1.45    |

|                                                             |                                                             |
|-------------------------------------------------------------|-------------------------------------------------------------|
| 125 lbs./sq. in.—7,150 m. p. s.                             | 50 lbs./sq. in.—7,100 m. p. s.                              |
| 150 lbs./sq. in.—3,300 m. p. s.                             | 100 lbs./sq. in.—2,900 m. p. s.                             |
| 400 lbs./sq. in.—2nd and 3rd cartridges failed to detonate. | 150 lbs./sq. in.—2,050 m. p. s.                             |
|                                                             | 300 lbs./sq. in.—2nd and 3rd cartridges failed to detonate. |

In the foregoing example the term "Blasting Soluble" nitrocellulose means the product of nitration of purified cotton cops by the pot process to a nitrogen content of 11.95 to 12.25%. The product is at least 95% soluble in ether alcohol solution and has a viscosity of 100 to 300 c. g. s. units in solution of three grams in 100 ml. acetone (95%) at 20° C.

What we claim is:

1. A gelatine blasting explosive comprising a porous vegetable material ingredient and an oxidising salt distributed through a continuous matrix of a liquid explosive nitric ester-nitrocellulose jelly, said porous vegetable material consisting of dried substantially protein-free, oil-free peanut meal.

2. A gelatine blasting explosive composition as claimed in claim 1 wherein the dried substantially protein-free, oil-free peanut meal is one made from peanuts from which the brown testa has first been removed.

3. A gelatine blasting explosive composition as claimed in claim 1 wherein the protein-free, oil-

free peanut meal is one which passes a 16 B. S. S. screen and is retained on a 100 B. S. S. screen.

4. A cartridge containing a gelatine blasting explosive comprising a porous vegetable material ingredient and an oxidizing salt distributed through a continuous matrix of a liquid explosive nitric ester-nitrocellulose jelly, said porous vegetable material consisting of dried substantially protein-free, oil-free peanut meal.

JAMES TAYLOR. 10  
JAMES V. GREGG.

## References Cited in the file of this patent

## UNITED STATES PATENTS

| Number      | Name                  | Date          |
|-------------|-----------------------|---------------|
| 5 1,895,144 | Botts et al. -----    | Jan. 24, 1933 |
| 1,965,731   | Woodbury -----        | July 10, 1934 |
| 1,992,189   | Chapman -----         | Feb. 26, 1935 |
| 2,129,367   | Williams et al. ----- | Sept. 6, 1938 |